

## UNITED STATES PATENT OFFICE

2,304,962

## FOG INHIBITOR FOR PHOTOGRAPHIC EMULSIONS

Samuel E. Sheppard and Waldemar Vanselow,  
Rochester, N. Y., assignors to Eastman Kodak  
Company, Rochester, N. Y., a corporation of  
New Jersey

No Drawing. Application October 9, 1941,  
Serial No. 414,284

10 Claims. (Cl. 95—7)

This invention relates to fog inhibiting agents for photographic emulsions and to photographic emulsions containing them.

Photographic emulsions, particularly ultra-sensitive emulsions are those containing color sensitizers exhibiting a tendency to fog. This fog manifests itself as a uniform deposit of silver extending over the emulsion. It may be caused by exposing the emulsion in a room which is not completely dark or by development of the film for protracted periods or at temperatures above normal. Highly sensitive emulsions are more likely to fog than those of lower sensitivity owing to the small amount of energy required to make the silver halide grains developable.

It is, therefore, an object of the present invention to provide photographic emulsions of enhanced stability and which do not exhibit a high tendency to fog. The compounds used for this purpose should not markedly lower the sensitivity of the light-sensitive materials in which they are incorporated.

The use of amino-substituted derivatives of pyrimidine as fog inhibitors is described in Kendall U. S. Patent 2,173,628, granted September 19, 1939, and in Davey & Knott U. S. application Serial No. 347,489, filed July 25, 1940, now Patent No. 2,273,562 of February 17, 1942. These patents do not describe the use of amino-substituted thiopyrimidines as fog inhibitors.

We have now discovered that 2-mercapto-pyrimidines having an amino substituent in the 4 position or 6-position or both of the pyrimidine ring are valuable fog inhibitors. The amino group may be a primary amino group or may be substituted with other groups.

2-mercapto-pyrimidine has the following structural formula:



Amino derivatives of this compound which we have found suitable as antifoggants are as follows:



In the preparation of an emulsion containing the anti-foggants used according to our invention, a solution of the fog inhibiting agent was made up in a suitable solvent such as water or alcohol and this solution mixed with the emulsion. In the tests which we made, a high speed negative emulsion containing no sensitizing dyes or coating doctors and having a pH of 7.1 was used. Stock solutions of the fog inhibiting compounds were made and these were added to the emulsion in varying amounts. The emulsions were coated on glass plates, dried and incubated to obtain a substantial fog on the control plate

containing no fog inhibitor. Incubation was carried out at 48½° C. for a period of time sufficient to produce an appreciable amount of fog on the control plate. All of the plates were incubated for the same period of time.

The amount of fog inhibiting agent added to the emulsion is of importance since if too much of the fog inhibiting compound is added it may desensitize the emulsion. The exact amount that must be used varies without particular fog inhibiting compounds selected and with the type of emulsion used as regards grain size and alkalinity of the emulsion and ratio of the gelatin to silver halide. However, we have found that with gelatino silver halide developing-out emulsions the amount of anti-foggant will generally vary between about .001 gram and 1 gram of anti-foggant per 1000 cc. of emulsion.

The fog inhibiting agents which we have found to be satisfactory may be used in various kinds of photographic emulsions. In addition to being useful in ordinary non-color-sensitized emulsions, they may also be used in ortho-chromatic or panchromatic emulsions or in X-ray emulsions. They can be used with or without sensitizing dyes and if used with sensitizing dyes may be added to the emulsion before or after such dyes.

The following table will serve to illustrate the amounts of the various specific fog inhibiting agents referred to above which we have found to be especially satisfactory. In each case the amount of fog inhibiting agent specified is used in 1000 cc. of gelatino silver halide emulsion containing from 5% to 10% gelatin and the table indicates the solvent in which each of the agents was incorporated in the emulsion:

| Compound | Grms./1,000<br>cc. emul-<br>sion | Solvent     |
|----------|----------------------------------|-------------|
| 1.       | .0036                            | Water.      |
| 2.       | .003                             | Water+NaOH. |
| 3.       | .00726                           | Water+KOH.  |
| 4.       | .081                             | Water+NaOH. |
| 5.       | .0094                            | Water.      |
| 6.       | .008-08                          | Water+NaOH. |
| 7.       | .008                             | Water+KOH.  |
| 8.       | .0035                            | Alcohol.    |
| 9.       | .001                             | Water.      |
| 10.      | .0077                            | Alcohol.    |

It is to be understood that more or less of the fog inhibiting agent than the amount indicated in the table above may be used. Generally, however, if a much greater amount is used in the

emulsion either no increased fog inhibiting effect is obtained or there is a marked decrease in sensitivity of the emulsion.

It is to be understood that we consider as included within our invention all modifications and equivalents falling within the scope of the appended claims.

We claim:

1. A photographic emulsion comprising a colloidal material having a sensitive silver salt dispersed therein and containing a 2-mercapto pyrimidine having an amino group in at least one of the positions in the pyrimidine ring, selected from the 4-position and the 6-position, in fog-inhibiting amount.
2. A photographic emulsion comprising a colloidal material having a sensitive silver salt dispersed therein and containing a 2-mercapto pyrimidine having a primary amino group in at least one of the positions in the pyrimidine ring, selected from the 4-position and the 6-position, in fog-inhibiting amount.
3. A photographic emulsion comprising a gelatino-silver halide emulsion containing a 2-mercapto-6-amino-pyrimidine in fog-inhibiting amount.
4. A photographic emulsion comprising a gelatino-silver halide emulsion containing a 2-mercapto-4-amino-pyrimidine in fog-inhibiting amount.
5. A photographic emulsion comprising a gelatino-silver halide emulsion containing a 2-mercapto-4,6-diamino-pyrimidine in fog-inhibiting amount.
6. A photographic emulsion comprising a gelatino-silver halide emulsion containing from about 0.001 gram to about 1 gram per liter of emulsion of a 2-mercapto-6-amino-pyrimidine.
7. A photographic emulsion comprising a gelatino-silver halide emulsion containing from about 0.001 gram to about 1 gram per liter of emulsion of a 2-mercapto-4-amino-pyrimidine.
8. A photographic emulsion comprising a gelatino-silver halide emulsion containing from about 0.001 gram to about 1 gram per liter of emulsion of a 2-mercapto-4,6-amino-pyrimidine.
9. A gelatino-silver halide emulsion containing a fog-inhibiting amount of 4,6-diamino-2-mercapto-pyrimidine.
10. A gelatino-silver halide emulsion containing a fog-inhibiting amount of 4-amino-6-hydroxy-2-mercapto-pyrimidine.

SAMUEL E. SHEPPARD.  
WALDEMAR VANSELOW.